

2,929,698

## EXPLOSIVE

Ludwig F. Audrieth and George C. Hale, Dover, N.J.

No Drawing. Application August 15, 1944  
Serial No. 549,599

1 Claim. (Cl. 52—5)

(Granted under Title 35, U.S. Code (1952), sec. 266)

The invention described herein may be manufactured and used by or for the Government for governmental purposes without the payment to us of any royalty thereon.

The present invention relates to a new explosive composition. More particularly the invention is based upon the discovery that certain salts of diaminoguanidine are explosives having highly favorable properties which make them of value for military or other uses. Such explosive compounds are represented by the type formula:



where HX represents any one of a series of inorganic or organic acids which will impart explosive properties to diaminoguanidine when combined with it.

While it is recognized that the acid derivatives of guanidine have been considered previously for use in explosives mixtures, we have found that they do not possess the favorable properties of the diaminoguanidine salts and, in fact, have not been used as military or industrial explosives so far as is known, due largely to the extreme insensitivity to the compounds. We have discovered that the sensitivity of the diaminoguanidine salts is such that they can be readily brought to complete high order detonation by a priming charge of mercury fulminate, whereas the corresponding salts of guanidine cannot be so detonated when tested under the same conditions. Evidently, the replacement of two amino groups in guanidine by hydrazino groups to produce diaminoguanidine (see structural formulas I and II) has a marked effect in increasing the sensitivity of the salts, i.e., the ease in which the salts can be made to explode.

I. Guanidine



II. Diaminoguanidine



This is considered an important discovery as no reference to such an effect has yet been encountered in the field of explosives. It is of definite interest that these new, more explosive salts of diaminoguanidine can be used alone as high explosives.

In addition to the favorable sensitivity to detonation of the diaminoguanidine salts, they have been found to be highly stable and to have power or brisance comparable to trinitrotoluene and to other explosives which have found extensive use as military explosives.

The more important and significant explosive characteristics of representative inorganic and organic salts of

diaminoguanidine, as determined by standard methods, are summarized in the following table:

|    |                                                                                | Diaminoguanidine |         |
|----|--------------------------------------------------------------------------------|------------------|---------|
|    |                                                                                | Nitrate          | Picrate |
| 5  | Melting Point, ° C.                                                            | 142-4            | 188-90  |
|    | Sensitivity to impact, Bureau of Mines App. using a 2 kg. wt., cm.             | 40               | 80      |
| 10 | Sand Test value, g. sand when initiated with 0.3 g. mercuric fulminate.        | 27.8             | 40.6    |
|    | Stability, cc. gas evolved by a 5 g. sample in the 120° Vacuum Stability Test. | 1.92             | 0.48    |
|    | Explosion Temperature, ° C.                                                    | 290              | 250     |

While we cite here only the nitrate and picrate of diaminoguanidine, we do not wish to be limited to these two salts, for we have found that such acids as perchloric, chloric, hydrazoic, styphnic, dinitrophenol, and dinitroresorcinol will combine with the base to give explosive products.

20 To emphasize the favorable properties of these compounds as explosives, the following comparisons are made. The impact sensitivity of tetryl and of pentaerythritol tetranitrate is given by the values 17 cm. and 26 cm. respectively, indicating that both the nitrate and picrate of diaminoguanidine are appreciably less sensitive to impact and therefore much safer to handle than these widely used high explosives. The sand test values, generally recognized by those skilled in the art as a measure of the brisance or shattering effect of an explosive, place these compounds in the same class with trinitrotoluene and the amatols.

25 Since the sand test values for the nitrate and picrate of diaminoguanidine are obtained through initiation by 0.3 g. of mercuric fulminate, it is furthermore indicated that these explosives can easily be made to detonate at high order and at a high rate. Particularly favorable and of utmost importance in determining the feasibility of using for military and commercial purposes such explosives is the stability of diaminoguanidine compounds. In fact the data indicates that the compounds cited above as examples are remarkably stable in that heating for 48 hours in a vacuum at 120° C. causes only negligible decomposition as evidenced by the small quantity of gas evolved in the test. By comparison, these compounds possess stability approaching that of trinitrotoluene and are more stable than tetryl and pentaerythritol tetranitrate, all of which are important military high explosives.

30 The diaminoguanidine compounds can be shown by calculation to yield relatively low temperature on explosion, and would therefore offer advantage over many other high explosives where a "cool" explosive is desired. Diaminoguanidine compounds, in particular the nitrate, can also be used as components of mixed explosives. We have found (a) that an explosive consisting of a 50/50 mixture of diaminoguanidine nitrate plus trinitrotoluene possesses greater power and brisance than the widely used composite of ammonium nitrate and trinitrotoluene; and (b) that such a mixture in the molten state can be cast loaded into shell, bombs, mines, and other devices used for blasting and demolition purposes to yield an excellent high explosive of high power and superior stability.

35 Having thus described the invention, what is claimed as new is:

An explosive composition consisting essentially of a diaminoguanidine salt of an acidic agent selected from the group consisting of nitric acid, picric acid, perchloric acid, chloric acid, hydrazoic acid, styphnic acid, dinitrophenol and dinitroresorcinol, and a detonating agent for detonating said salt.

(References on following page)

3

References Cited in the file of this patent

## UNITED STATES PATENTS

1,312,464 Woodbury ----- Aug. 5, 1919  
1,758,169 Olsen ----- May 13, 1930

## FOREIGN PATENTS

12,617 Great Britain ----- 1901

4

## OTHER REFERENCES

Davis: "Chemistry of Powder and Explosives," II,  
pages 280-81 (1943).  
Beilstein: "Handbuch der Organische Chemie," vol.  
VI (4th ed.), page 279.  
Beilstein: "Handbuch der Organische Chemie," vol.  
III (1st sup. to the 4th edition), page 57.